

March 28, 1961

E. J. GRISSET, JR., ET AL

2,977,184

PRODUCTION OF RAYON

Filed June 16, 1953

5 Sheets-Sheet 1



INVENTORS  
ERNEST J. GRISSET, JR.<sup>44</sup>  
GILBERT I. THURMOND

BY

*Met R. Poston*

ATTORNEY

March 28, 1961

E. J. GRISSET, JR., ET AL

2,977,184

PRODUCTION OF RAYON

Filed June 16, 1953

5 Sheets-Sheet 2



Fig. 2.



Fig. 3.

INVENTORS

ERNEST J. GRISSET, JR.<sup>44</sup>  
GILBERT I. THURMOND

BY

*Met R. Boston*

ATTORNEY

March 28, 1961

E. J. GRISET, JR., ET AL

2,977,184

PRODUCTION OF RAYON

Filed June 16, 1953

5 Sheets-Sheet 3



INVENTORS

ERNEST J. GRISET, JR. AND  
GILBERT I. THURMOND

BY

*Met R. Boston*

ATTORNEY

March 28, 1961

E. J. GRISET, JR., ET AL

2,977,184

PRODUCTION OF RAYON

Filed June 16, 1953

5 Sheets-Sheet 4



INVENTORS

ERNEST J. GRISET, JR.<sup>440</sup>  
GILBERT I. THURMOND

BY

*Mer R. Poston*

ATTORNEY

March 28, 1961

E. J. GRISET, JR., ET AL

2,977,184

## PRODUCTION OF RAYON

Sheets-Sheet 5

Filed June 16, 1953 5 Sheets-Sheet 5



ERNEST J. GRISSET, JR. AND  
GILBERT I. THURMOND

*Met R. Poston*  
ATTORNEY

# United States Patent Office

2,977,184

Patented Mar. 28, 1961

1

2,977,184

## PRODUCTION OF RAYON

Ernest J. Griset, Jr., and Gilbert I. Thurmond, Asheville, N.C., assignors to American Enka Corporation, Enka, N.C., a corporation of Delaware

Filed June 16, 1953, Ser. No. 362,016

4 Claims. (Cl. 18—54)

This invention relates to the treatment of filamentous material such as threads, filaments, fibers, yarns and the like, hereinafter referred to generically as threads; and more particularly to a method for the continuous production of freshly spun viscose rayon threads having improved properties. In its more specific aspects, the invention relates to a method for continuously spinning improved high tenacity rayon threads in a tube spinning system.

In U.S. Patent No. 2,725,276, there are disclosed a method and apparatus for producing synthetic threads by the so-called Griset tube spinning method. The present invention utilizes the concept of tube spinning disclosed in the latter case in the manufacture of high tenacity viscose rayon. An entirely new machine which incorporates the Griset tube spinning principle has been developed for the production of high tenacity viscose rayon threads. This apparatus is the subject matter of copending application Serial No. 361,892, filed June 16, 1953. The present application is concerned primarily with the method for producing improved high tenacity thread in this apparatus.

It is an object of the present invention to provide a method for utilizing the Griset tube spinning principle to produce viscose rayon thread having improved properties.

A further object of this invention is to provide a continuous tube spinning process for the production of high tenacity viscose rayon threads.

A still further object of the invention is to produce a continuous high tenacity viscose rayon thread having improved physical properties.

Other objects and advantages of the invention will be apparent upon consideration of the following detailed description.

In general, the present invention comprises a process for producing a high tenacity viscose rayon thread wherein the conditions in the spinbath, in the aftertreating zones, and during the final drying operation, are carefully controlled, all of which will be more fully described hereinafter.

In accordance with the present invention, viscose is extruded into filamentary material in an acid coagulating and regenerating bath containing between 6.5 and 8.0% sulfuric acid and maintained preferably at a temperature of at least 65° C. Thereafter, the resultant partially regenerated filamentary material is stretched between 50 and 100% and subjected to an aftertreatment while propelling it successively through a series of spaced, generally horizontally disposed confined liquid treating zones solely by means of a flowing liquid in each zone. Thereafter, the said material is dried, rewet, restretched and redried under tension. Since the process of the present invention is carried out in an extremely short time, it is surprising that the viscose rayon thread obtained has properties in most instances better than thread produced according to conventional methods.

2

The invention will be further explained by reference to the annexed drawings, wherein

Figure 1 is a section in side elevation of part of the spinning machine used in the present invention;

5 Figure 2 is a plan view of a group of treating tubes used for a single spinning position;

Figure 3 is a view in side elevation of the group of treating tubes shown in Figure 2;

10 Figure 4 is a perspective view of the back side of a spinning machine used in the present invention;

Figure 5 is a side elevation of the drying assembly used in the present invention; and

Figure 6 is a diagrammatic flow sheet of the liquid circulation system used in the invention.

15 Referring now to Figure 1, viscose solution is extruded through spinneret 10 into acid coagulating bath 11 to produce thread 12. The thread 12 is wrapped several times around small godet 13, passed downwardly to roller 14 and then upwardly to large godet 15 where it is also wrapped several times around. The peripheral speeds of the two godets are adjusted so as to impart a stretch of about 75% to the thread. Roller 14 is submerged in a second bath 16 and the thread 12 passes through this bath 16 during its travel between small godet 13 and large godet 15. It will thus be apparent that the stretching of the thread 12 occurs just before, during and after the time that it is being subjected to the treatment of the second bath 16.

20 Upon leaving the large godet 15, the thread 12 is 30 passed downwardly and is intercepted by a stream of liquid issuing from jet 17 by which it is propelled into and through a treating tube 18. A detailed description of the manner in which the thread 12 is initially spun in and introduced into the tube 18 will not be given here inasmuch as this procedure is fully described in U.S. Patents Nos. 2,675,690 and 2,725,276, to each of which reference is hereby made.

25 Upon leaving the tube 18, the thread 12 is 35 discharged into a jet box 19. The thread entering the box 19 from the tube 18 first passes along deflector 20 and then it is liquid propelled in succession through treating tube 21, deflector 22, tube 23, deflector 24, tube 25, deflector 26, tube 27, deflector 28, tube 29, deflector 30, tube 31, deflector 32 and finally tube 33.

30 The deflectors 20, 24, 28 and 32 are mounted on a bar 34 for laterally shifting to and from a position registering with the entrance ends of tubes 21, 25, 29 and 33, respectively (see Figure 2). Deflectors 22, 26 and 30 are mounted on a bar 35 similar in structure and function

40 to the bar 34. It will be apparent from Figures 2 and 3 that separate liquid recovery compartments underlie the deflectors in registry with the exit end of the treating tubes. When spinning-in is completed each aftertreating tube, except tube 33, discharges into a compartment and each compartment has a drain by which the liquid recovered therein can be recycled. As seen in Figure 2, the thread reverses its direction of travel at the end of each tube. While passing through these eight treating tubes, the thread is not only conveyed

45 by the liquid but is subjected to treatment with the conveying liquid to complete the regeneration of the viscose thread. Referring now to Figure 3, supply headers 18a, 21a, 23a, 25a, 27a, 29a, 31a and 33a furnish liquids to the corresponding treating tubes.

50 Inasmuch as the spinning-in and aftertreating operations in the tube assembly are more or less automatic, and manual handling of the thread during regeneration is not required, treating liquids having high temperatures may be employed. For example, treating liquids having a temperature of 90° C. have been employed in the above-described tube treating process. The use of these ex-

cessively hot treating solutions in one factor contributing to a reduction in the total time required for completely regenerating the viscose rayon thread. The thread passes through the entire aftertreating system in a remarkably short time. For example, at a spinning speed of about 76 meters per minute, it has been found that the thread passes through eight treating tubes 32 inches in length in around seven seconds. In view of the fact that not more than seven or eight seconds are required for the thread to pass from the initial spinning bath 11 through the stretching operation and into the first treating tube 18, the total time required for transforming viscose solution into a substantially completely regenerated and finished viscose rayon thread is less than twenty seconds. Considering the manifold physical and chemical changes which occur during this transformation, the shortened treating time is indeed phenomenal.

It is important to note that the abbreviated treating time mentioned above is not achieved by the use of high temperatures alone. An even more important factor is the tension condition of the thread during the aftertreatment. Since the thread is conveyed through the treating tubes solely by the passage of the liquid flowing through the tubes, it is subjected to a negligible tension during the time it is being aftertreated. The tension on the thread 12 is only about 10 grams as it enters tube 18 and it has been found that this tension does not change appreciably as the thread proceeds through the other tubes. By observation it is apparent that the thread in the tubes is in a substantially relaxed condition; the filaments are fully separated and dispersed with the liquid freely penetrating between them. This relaxed condition of the yarn is of primary importance in the practicing of the present invention.

In a typical aftertreating arrangement tube 18 is supplied with water containing 0.16%  $H_2SO_4$  at 90° C., tube 21 is supplied with 4% sulphuric acid at 90° C., tube 23 with water containing 0.1% sulphuric acid at 90° C., tube 25 with water at 90° C., tube 27 with 0.09% sodium bicarbonate at 90° C., tubes 29 and 31 with water at room temperature and tube 33 with 1% "Nopco" at room temperature. Even without a specific desulphurization treating liquid the sulphur content of the treated thread is abnormally low, usually less than 0.05%. The high degree of sulphur removal is believed to be at least partly due to the dispersed condition of the individual filaments during aftertreatment.

The term "Nopco" as used herein refers to a finishing solution sold by Nopco Chemical Co., Harrison, N.J., under the trade name "Nopco 2169-M," containing mineral oil blended with emulsifying materials.

Upon passing from the exit end of tube 33, the thread 12 and the finishing solution empty into extension tube 36 and are carried to a position above trough 37. The finishing solution falls into trough 37 and is carried away for recirculation. The thread 12 leaving the extension tube 36 is guided through combs generally indicated with the numeral 38 in Figure 4, in a path parallel with, but overlying, trough 37 to the end of the spinning machine where it is drawn off in warp form by means of draw rolls 39. The manner in which the various threads issuing from the finishing tube extensions are brought together for the purpose of forming a warp sheet, is believed to be obvious from Figure 4. For a more detailed explanation of the method for forming the warp sheet, reference is made to U.S. Patent No. 2,789,339.

Referring now to Figure 5, the warp of threads passing through draw rolls 39 is brought into contact with a first series of rotating drying cylinders 40-51 inclusive. The completely dried threads leaving the cylinder 51 are passed via freely rotatable rollers 52 and 53 into a bath of "Nopco" finishing solution contained in slasher pan 54, through driven squeeze rolls 55, 56, 57, and to a second series of drying cylinders 58-69, inclusive. The sec-

ond series of drying cylinders 58-69, inclusive, are preferably operated at a speed slightly in excess of squeeze rolls 55, 56, 57, to impart an additional stretch to the once dried threads. On leaving the final drying cylinder 69, the warp of threads is passed to any suitable take-up for a continuously running filamentary material.

The propulsion of the drying cylinders 40-51, inclusive, is effected by a driving chain 70 which interconnects the cylinders, the drive being imparted to the system 10 through a sprocket 71 coaxial with drying cylinder 44. Sprocket 71 is driven from a chain 72 which in turn is driven from a transmission system generally designated by numeral 73. Drying cylinders 58-69, inclusive, are similarly driven by an interconnecting chain 74 and power is supplied to the group through a sprocket 75 coaxial with cylinder 65.

Upon reference to Figure 6 a typical liquid circulation system for aftertreating tire yarn can be seen. In that figure the supply and exhaust manifolds are represented 20 as blocks and all of the seventy-two tubes through which the liquids pass from one manifold to the other are represented by a single solid line numbered to correspond to the appropriate treating tube of Figure 2.

Beginning then with the tubes 18, it is seen that they 25 are supplied with hot water from a tank S-1 and that manifold 18b drains to sewer. Water is supplied to tank S-1 through a temperature control heater 76 by a pump 77 which draws from a recovery tank R-1 which receives from manifold 23b the discharge from tubes 23. 30 Tubes 23 are supplied from manifold 23a which is fed from tank S-3. Tank S-3 is supplied by a pump 78 which delivers water from recovery tank R-3 through a temperature control heater 79. The water in tank R-3 is recovered from manifold 25b by tubes 25. Tubes 25 35 are supplied from a tank S-4 through manifold 25a. The tank S-4 receives its water through a heater element 80 from a pump 81 drawing from a tank R-4. Tank R-4 is supplied from manifold 29b which is fed by tubes 29 which in turn are supplied by manifold 29a. Manifold 29a is supplied from tank S-6 which is fed from tank R-6 by a pump 82 delivering through a heater element 83. Tubes 31 are supplied with fresh soft water heated to the proper temperature. This water is discharged from tank S-7 through manifold 31a. The recovery from tubes 31 is received in manifold 31b and delivered to recovery tank R-6.

It can now be seen that for treating tire yarn the first, third, fourth, sixth and seventh tubes of each group may 50 contain water. The water which first contacts the newly spun yarn has already contacted yarn on four previous occasions and it is not until the fifth water treatment that the yarn encounters fresh water.

In the second tube of each group, the tubes 21, the 55 yarn is treated with sulphuric acid supplied to tank R-2 and delivered from it by pump 84 through heat control element 85 to supply tank S-2. The tank S-2 feeds manifold 21a and the recovery manifold 21b feeds back to tank R-2. Make-up liquid is supplied to tank R-2 as indicated in Figure 6.

The fifth tubes of each group, tubes 27, are supplied 60 with  $NaHCO_3$  by a system identical to acid supply system for tubes 21. Sodium bicarbonate recovered from manifold 27b is discharged into tank R-5 from which pump 86 delivers it through a heat control element 87 to tank S-5. From supply tank S-5 the sodium bicarbonate is delivered to manifold 27a.

The only other solution is finishing solution which is 65 delivered from the tank S-8 to the tubes 33 from the manifold 33a. This solution is not recovered in a manifold at all but passes from the tubes 33 through the large tubes 36 into the trough 37. The finishing solution stays with the yarns as they move along the trough during spinning-in and it moves parallel to the warp of yarns running above the trough 37 during the remainder of the

doff. At the end of the trough 37, the finishing solution is discharged to a screened tank marked R-8 in Figure 6. From the recovery tank, to which make-up may be added through line 88, a pump 89 delivers the solution to tank S-8. If further finish is supplied to the yarns while they are being dried running as a warp, the slasher pan 54 may be supplied in parallel with the tubes 33 as can be seen in Figure 6.

In Figure 6 all of the supply tanks are shown as above the recovery tanks. The supply tanks are disposed higher than the tube groups to give a uniform head or pressure at the supply manifolds which, in turn, results in uniform flow through the tubes. By arranging the heaters between the recovery tanks and the supply tanks, the likelihood of entraining air is reduced.

#### Example I

A viscose solution containing 7.3% cellulose, 6.8% caustic, 2.25% sulphur, and having an ammonium chloride number of 11.5, was extruded into a spinbath containing 7.2% sulphuric acid, 17% sodium sulphate, 3.4% zinc sulphate, and 26 p.p.m. lauryl pyridinium chloride to produce a thread of 1650 denier, 720 filaments. The temperature of the spinbath was 70° C. The coagulated thread was passed up and around small godet 13 and then back down under roller 14 submerged in a second bath containing 2.5% sulphuric acid at 90° C. Upon leaving the second bath, the thread was passed to large godet 15 driven at a speed faster than godet 13 with the result that a stretch of about 75% was imparted to the thread between the small godet 13 and the large godet 15.

The thread was next passed at a speed of about 76 meters per minute through a series of eight treating tubes by means of a jet of liquid introduced at the entrance end of each tube. While being propelled through the eight treating tubes, the thread was subjected to treatment with the following liquids in the order given: recycled water containing 0.16% H<sub>2</sub>SO<sub>4</sub> at 90° C., 4% sulphuric acid at 90° C., recycled water containing 0.1% H<sub>2</sub>SO<sub>4</sub> at 90° C., recycled water at 90° C., 0.09% sodium bicarbonate at 90° C., recycled water at 90° C., water at 90° C., and finishing solution at room temperature. The term "recycled water" used in reference to the treating liquids refers to water which had been used in at least one previous treating step without subsequent purification. The thread leaving the tube containing the finishing solution was drawn off in a warp sheet of similarly treated threads by means of draw rolls 39. The warp sheet was stretched about 1% and dried by passing it into contact with a first series of steam heated drying cylinders. The dried warp was stretched about 4% more during which time it was re-wet by passage through bath 54. The warp of threads was withdrawn from the bath 54 by means of driven squeeze rolls 55, 56, 57, and passed to a second series of drying cylinders rotating at a speed sufficient to impart about 1% additional stretch to the threads between the squeeze rolls 55-57 and the second series of drying cylinders. The re-dried threads were taken up in package form on a winding machine. The thread produced had the following properties:

|                                 |      |
|---------------------------------|------|
| Dry strength, gms./100 denier   | 334  |
| Dry elongation-total, percent   | 12.6 |
| Cond. strength, gms./100 denier | 282  |
| Cond. total elongation, percent | 15.4 |
| U.S. Rubber fatigue             | 512  |

#### Example II

A viscose solution similar to the one used in Example I was extruded into a spinbath of the composition given in Example I. The coagulated thread of 1650 denier, 720 filaments, was stretched about 70% in a second bath containing dilute sulphuric acid at 90° C.

The thread was aftertreated by passing it through a series of six treating tubes by means of a jet of liquid introduced into each tube. The thread passing through

the tubes was subjected to treatment with the following liquids in the order given: recycled water containing 0.16% H<sub>2</sub>SO<sub>4</sub> at 90° C., 4% sulphuric acid at 90° C., recycled water containing 0.1% H<sub>2</sub>SO<sub>4</sub> at 90° C., recycled water at 90° C., 0.09% sodium bicarbonate at 90° C., and water at 90° C. The thread leaving the sixth tube was drawn off in a warp sheet of similarly treated threads and re-stretched and double dried according to the conditions given in Example I. The re-dried threads were taken up in package form on a winding machine and had the following properties:

|                                 |      |
|---------------------------------|------|
| Dry strength, gms./100 denier   | 343  |
| Dry elongation-total, percent   | 11.9 |
| Cond. strength, gms./100 denier | 285  |
| Cond. total elongation, percent | 14.1 |
| U.S. Rubber fatigue             | 528  |

It has been found that the double drying procedure used in the above examples definitely contributes to superior properties in the finished thread. Samples of thread produced in a similar process involving only a single drying step at times equaled in physical properties the thread produced by the double drying procedure. However, in general, better strength and more uniform strength was found in thread produced with the double drying technique. The fatigue values were also better in the double dried thread.

In order to obtain the most favorable results it is desirable to carefully control the acid concentration in the spinbath while at the same time controlling the ratio between the acid concentration and the salt concentration in the spinbath. Calculating the acid/salt ratio as

$$\frac{\text{total weight of sulphuric acid}}{\text{total weight of sodium sulphate}}$$

it is desirable that the ratio be maintained within the limits 0.35 to 0.50, and preferably at a ratio of about 0.42. While maintaining the foregoing ratio, the best quality threads are obtained when the acid concentration in the spinbath is held within the range of 6.5% to 8.0% sulphuric acid. At acid concentrations below 6.5% the fiber quality of the high tenacity thread becomes markedly inferior. When the acid concentration is appreciably higher than 8.0% the desired physical properties are difficult to obtain.

Therefore, by calculating the sodium sulphate content from the above formula, it is seen that the sodium sulphate should be between 13-23% with the preferred range being 16-19%.

What is claimed is:

1. A process for continuous production of viscose rayon thread comprising the steps of extruding viscose into filamentary material in an acid coagulating and regenerating bath containing between 6.5 and 8.0% sulfuric acid and maintained at a temperature of at least 65° C., stretching the resultant partially regenerated filamentary material between 50 and 100% and subjecting the said material to an aftertreatment while propelling it successively through a series of spaced generally horizontally disposed confined liquid treating zones solely by means of a flowing liquid in each zone, the after treating liquids in at least four of said zones being maintained at a temperature of at least 70° C. with said material being exposed to said liquids for a total time of not more than 30 seconds, whereby a high tenacity thread is produced.

2. A process for continuous production of viscose rayon thread comprising the steps of extruding viscose into filamentary material in an acid coagulating and regenerating bath containing between 6.5 and 8.0% sulfuric acid and maintained at a temperature of at least 65° C., stretching the resultant partially regenerated filamentary material between 50 and 100%, subjecting the said material to an aftertreatment while propelling it successively through a series of spaced generally horizontally disposed confined liquid treating zones solely by means of a flow-

ing liquid in each zone, and thereafter drying, rewetting and redrying said treated filamentary material, the after-treating liquids in at least four of said zones being maintained at a temperature of at least 70° C. with said material being exposed to said liquids for a total time of not more than 30 seconds, whereby a high tenacity thread is produced.

3. A process for continuous production of viscose rayon thread comprising the steps of extruding viscose into filamentary material in an acid coagulating and regenerating bath containing between 6.5 and 8.0% sulfuric acid and maintained at a temperature of at least 65° C., stretching the resultant partially regenerated filamentary material between 50 and 100%, subjecting the said material to an aftertreatment while propelling it successively through a series of spaced generally horizontally disposed confined liquid treating zones solely by means of a flowing liquid in each zone, and thereafter drying said treated filamentary material under tension, rewetting and redrying said treated filamentary material, the aftertreating liquids in at least four of said zones being maintained at a temperature of at least 70° C. with said material being exposed to said liquids for a total time of not more than 30 seconds, whereby a high tenacity thread is produced.

4. A process for continuous production of viscose rayon thread comprising the steps of extruding viscose into filamentary material in an acid coagulating and regenerating bath containing between 6.5 and 8.0% sulfuric acid and between 16 and 19% sodium sulfate and maintained at a temperature of at least 65° C., stretching the resultant partially regenerated filamentary material be-

5 through a series of spaced generally horizontally disposed confined liquid treating zones solely by means of a flowing liquid in each zone, said aftertreatment including the steps of washing the filamentary material with water maintained at a temperature of at least 70° C., treating the filamentary material with dilute sulfuric acid and treating the filamentary material with a solution of sodium bicarbonate, applying a finish solution to the treated material, thereafter drying said material under tension, rewetting, and redrying said filamentary material under tension, the aftertreating liquids in at least four of said zones being maintained at a temperature of at least 70° C. with said material being exposed to said liquids for a total time of not more than 30 seconds, whereby a high tenacity thread is produced.

20 References Cited in the file of this patent

UNITED STATES PATENTS

|           |                  |               |
|-----------|------------------|---------------|
| 1,427,238 | Sinkwitz         | Aug. 29, 1922 |
| 1,871,100 | Walton et al.    | Aug. 9, 1932  |
| 2,203,793 | Lovett           | June 11, 1940 |
| 2,348,415 | Polak            | May 9, 1944   |
| 2,369,191 | Thurmond         | Feb. 13, 1945 |
| 2,491,938 | Schlosser et al. | Dec. 20, 1949 |
| 2,725,276 | Griset           | Nov. 29, 1955 |
| 2,725,277 | Rilling et al.   | Nov. 29, 1955 |